

## UNITED STATES PATENT OFFICE

WILLIAM H. HAMPTON AND BRUCE B. FARRINGTON, OF BERKELEY, CALIFORNIA, ASSIGNEES, BY MESNE ASSIGNMENTS, TO STANDARD OIL COMPANY OF CALIFORNIA, OF SAN FRANCISCO, CALIFORNIA, A CORPORATION OF DELAWARE

## IMPROVED PETROLEUM PRODUCT AND ART OF WOOD PRESERVATION

No Drawing. Application filed December 19, 1923, Serial No. 681,470. Renewed November 26, 1929.

This invention relates to the preparation of a new petroleum product and particularly to the art of timber preservatives and has to do especially with the preservation of piling and other timbers from the attack of marine insects and *Teredos* and from fungi or other wood-destroying organisms.

An object of the present invention is to produce a novel acid sulfur oil or oils from petroleum.

An object of this invention is to prepare from a petroleum oil, or from products derived therefrom, a timber preservative which shall have properties, including toxicity and impregnation of wood, substantially equivalent to those of the well-known and widely used timber preservative called creosote.

Another object is to prepare such a timber preservative at a cost sufficiently low that its manufacture will be commercially and economically feasible.

Heretofore, when petroleum oils or products therefrom have been used for the preservation of timbers, they have been used either as paints, water-proofing agents and the like, or they have been used as carrier agents or diluents for preservatives, the poisonous and antiseptic agents of which having been derived from some other source.

We have discovered that both the toxic agent and the carrier agent or diluent, can be prepared from petroleum products, whereby a timber preservative is obtained having a toxicity, as well as other desirable properties, substantially equivalent to those of creosote.

In addition to the naphthenic acids which occur in some petroleum oils, for example, in Russian oils, California oils, etc. there exist in petroleum oils other and more complex organic compounds of an acid sulfur character whose nature is not well understood and which vary both in different petroleum oils and in the distillates derived therefrom.

These compounds we herein term "acid sulfur oils." These "acid sulfur oils" we employ as the toxic agent for our timber preservative.

The timber preservative which this invention

comprises, is made up of substantially 5% or more of these acid sulfur oils mixed with approximately 95% or less of a carrier agent or diluent, which carrier agent may be any ordinary fuel oil or petroleum distillate. A fuel oil which will give a resulting mixture, having the same viscosity as creosote, is preferable, though not necessary.

We prefer to make use of a group of "acid sulfur oils" which occur in petroleum distillates which have been obtained from a pressure distillation or "cracking" operation. The acid sulfur oils obtained from such distillates respond to several chemical reactions which, instead of being characteristic of the acid oils naturally occurring in petroleum, are typical of phenolic bodies. Such acid sulfur oils possess toxic properties to a somewhat greater degree than those naturally occurring in petroleum oils.

These "acid sulfur oils" have a decided toxic property toward fungi and wood-destroying organisms in general. A solution of these "acid sulfur oils" in a carrier or diluent comprising an ordinary fuel oil or petroleum distillate forms an effective timber preservative having substantially all of the properties which are desirable and effective as a timber preservative in creosote. This solution may be applied to timbers in the same manner as creosote. No "bleeding" or exudation from the wood occurs and after being processed with this solution, the wood is immediately available for service.

The following is given as an example of a preferred process by which we extract these acid sulfur oils and employ them for the preparation of a timber preservative.

To a petroleum distillate, which has been obtained from a pressure distillation or "cracking" operation, we add a sufficient quantity of lye to neutralize the acid sulfur oils of the distillate, after which the resulting lye sludge is separated from the distillate. Fuel oil, amounting to approximately 50% by volume of the recoverable acid sulfur oils is then added to the lye sludge, after which it is neutralized with a mineral acid, for example, sulphuric acid, allowing to settle, and the aqueous layer drawn off and discarded.

The oil, thus separated and containing the desired acid sulfur oils, is washed with water after which it is mixed with sufficient quantity of fuel oil to give a mixture of the desired strength. Approximately 15% of the product obtained after the washing with water will, when mixed with approximately 85% of fuel oil, result in a preservative having substantially 10% of the toxic acid sulfur oils, the balance being carrier oil. A mixture of such proportions has been found to approximate very closely all the desirable and effective properties of creosote. Other mixtures in which there is more or less of the toxic acid sulfur oils may of course be used.

In the procedure as outlined above, a portion of the total quantity of fuel oil used is added to the lye sludge before the same is neutralized with sulphuric acid. This is done to prevent the acid sulfur oil from holding up a large quantity of water, which it would do otherwise, and to minimize any loss due to the slight solubility of the acid sulfur oils in water. The addition of a part of the carrier oil, at this point, is however, optional. Obviously the addition of all the carrier oil used may, if desired, be made when the final mixing to the desired strength of toxic ingredient takes place.

30 By employing a distillate obtained from a pressure distillation operation, we may utilize a waste product which sometimes results from the treatment of such a distillate. In the treatment of a distillate obtained from a pressure distillation operation it is sometimes customary to employ a preliminary lye treatment prior to the sulphuric acid treatment of the distillate. When such lye treatment is used, the resulting lye sludge is a waste product and a great nuisance about a refinery. This waste product we use as a source of the acid sulfur oils for our timber preservative. It will therefore be seen that when such waste produced is employed the raw material cost for our toxic ingredient is very small and we are able to manufacture a timber preservative at a greatly reduced price.

Having thus described our invention, we claim:

50 1. A process of preparing a wood preservative containing a toxic compound derived from the distillates of a pyrogenetic process of cracking petroleum oils, which comprises adding sufficient lye solution to neutralize the acid sulfur compounds of such distillate, removing the lye sludge, adding mineral oil to said lye sludge, neutralizing the lye sludge with a mineral acid, thereby leaving the acid sulfur compounds in the mineral oil and in 55 a phase separate from the aqueous acid phase, and separating the oil phase from the acid phase.

2. A process of preparing a wood preservative containing toxic compounds produced 60 from products of pressure distillation or

cracking of petroleum oils, which comprises adding a lye solution to neutralize and separate the acid sulfur compounds from the products of the pressure distillation or cracking of petroleum oils, adding mineral 70 oil to the lye sludge in proportions of approximately 50% of the recoverable acid sulfur compounds, adding a mineral acid adapted to neutralize the lye sludge, separating the aqueous layer formed, washing the 75 oil and acid sulfur compounds with water, and adding further mineral oil to serve as a carrier of the toxic bodies.

3. A process of preparing a wood preservative from the products of pressure distillation or cracking of petroleum oils which comprises adding lye solution to said products to neutralize and separate the acid sulfur compounds, separating the lye sludge thus formed from the said products, adding 80 mineral oil in an amount equal to approximately 50% of the recoverable acid sulfur compounds, adding a solution of a mineral acid to neutralize the lye present, withdrawing the resultant aqueous layer from the resultant oil and acid sulfur compound layer, washing said latter layer with water, and finally adding additional mineral oil to act as a carrier of the acid sulfur compounds or toxic bodies.

4. A wood preservative containing toxic compounds, such toxic compounds being those derived from the distillates of a pyrogenetic process of cracking petroleum oils when said distillates are treated with sufficient lye solution to neutralize the acid sulfur compounds thereof and the resulting lye sludge is neutralized in the presence of a mineral oil with a mineral acid, the toxic compounds being the resultant acid sulfur 100 compounds which remain in the mineral oil, the wood preservative containing also a carrier.

5. A wood preservative consisting of acid sulfur toxic compounds, such as are derived 110 when a distillate of a pyrogenetic process of cracking petroleum oils is treated with sufficient lye solution to neutralize and separate the acid sulfur compounds from the products of pressure distillation, and mineral oil 115 is added to the resultant lye sludge in proportions of approximately 50% of the recoverable acid sulfur compounds in the presence of a mineral acid sufficient to neutralize the lye sludge, the acid sulfur toxic compounds being those compounds which remain in such added mineral oil when the lye sludge is separated therefrom, the wood preservative 120 also containing a carrier.

6. A process of preparing acid sulfur 125 compounds, similar to thiophenols or thionenols, from the distillates of a pyrogenetic process of cracking oils which comprises treating the distillates, still containing phenolic-like acid sulphur compounds, with lye 130

solution to neutralize the acid sulfur compounds, separating the lye sludge produced, neutralizing the lye sludge with acid and separating the aqueous layer from the resultant acid sulfur compounds.

7. An acid sulfur oil, similar to thiophenols and thioethenols, the same being derived from the distillates of a pyrogenetic process of cracking petroleum oil, containing phenolic-like acid sulphur compounds, when said distillates are treated with sufficient lye solution to neutralize the acid sulfur compounds thereof and the resulting sludge is neutralized in the presence of a mineral oil with a mineral acid, the acid sulfur oils being the resultant compound which remained in the mineral oil.

Signed at Richmond, California, this 11th day of December, 1923.

20 WILLIAM H. HAMPTON.  
BRUCE B. FARRINGTON.

25

30

35

40

45

50

55

60

65